

J. GLASSFORD.  
WATERPROOF MATERIAL.  
APPLICATION FILED JULY 31, 1907.

921,538.

Patented May 11, 1909.



Fig. 1.



Fig. 2.



Fig. 3.



Fig. 4.

WITNESSES:

G. H. Griffin  
L. Flynn

INVENTOR  
John Glassford  
BY  
Knight Bros.  
ATTORNEYS

# UNITED STATES PATENT OFFICE.

JOHN GLASSFORD, OF JERSEY CITY, NEW JERSEY, ASSIGNOR TO CONSOLIDATED WATER-PROOF COMPANY, OF NEW YORK, N. Y., A CORPORATION OF NEW YORK.

## WATERPROOF MATERIAL.

No. 921,538.

Specification of Letters Patent.

Patented May 11, 1909.

Application filed July 31, 1907. Serial No. 386,501.

*To all whom it may concern:*

Be it known that I, JOHN GLASSFORD, a citizen of the United States, and residing in Jersey City, Hudson county, New Jersey, have invented new and useful Improvements in Waterproof Material; and, in order that those skilled in the art may understand, make, and practice the said invention, I give the following specification thereof.

10 My invention relates to water proof material of the character employed for rendering such structures as subways, underground conduits, walls, foundations, pipe galleries or the like water proof. Heretofore water proof material of various kinds and structures have been employed for these purposes, but all such material with which I am acquainted, while water proof when first laid, rapidly deteriorates, loses its water 20 proof character and becomes useless. The main causes of this I have ascertained to be due to the fact that the material is not proof against the action of the soil or other surroundings in or near which it is laid. In 25 manufacturing districts and in cities many substances of various kinds, manufacturing wastes, etc., find their way into the soil which have a strong chemical or solvent action on known waterproofing material usually employed in subterraneous construction. Among these substances the principal are: what is known as "gas drip"—a condensation product coming from gas mains and pipes and containing the lighter hydrocarbons—benzole, benzin, kerosene, lubricating oils and other organic substances which exert a strong solvent action on the bituminous and asphaltic waterproofing material usually employed. Such fluids, or soil 35 drainage or seepage containing the same, coming in contact with ordinary waterproofing material rapidly penetrate the same and thereby destroy their waterproof properties and render the same useless. Another objection to water proofing material commonly used is that it becomes hard and brittle, and cracks and fissures form therein, particularly upon bending the same, and water and dampness penetrate the cracks 40 and fissures. A further defect in ordinary waterproofing material is that it requires the use of a fluid cement to secure the same to the walls, subway or foundation surfaces. This fluid cement is usually in the form of a molten asphalt, pitch, tar or the like or in the

form of a solution of such substances. Aside from the cumbrousness and the necessity of maintaining heating kettles for the former and the danger of fire and explosion from the inflammability of the latter, it is found that such fluid cements will not attach the material to a damp or wet wall or surface, and it is obvious that this is precisely the condition and situation that waterproofing material is employed to meet.

60 The object of my invention is to produce a waterproof material which is proof not only against water and dampness but against "gas drip" oils, and organic solvents in general, which preserves its toughness and flexibility and which will readily and firmly adhere to any surface wet or dry without the use of a hot or fluid asphaltic or similar cement.

65 In the accompanying drawing are illustrated several forms of the invention.

70 Figure 1 represents one form of the invention in sectional view, the plies and layers being exaggerated for the sake of clearness of illustration. Figs. 2, 3 and 4 are similar 75 views of other forms of the invention.

80 In all the views the same reference characters indicate corresponding features.

85 The water proofing material is preferably constructed according to my invention of a fabric such as paper, felt, burlap, or any suitable fabric, indicated at B in the drawing, which is saturated with bituminous composition, by passing the same through the heated composition in a suitable tank, or in any 90 other manner which may be convenient or desired. The object is to thoroughly impregnate and saturate the fabric with the composition. The composition employed for this purpose may be any suitable bituminous or asphaltic waterproofing composition usually employed for the purpose, and having a melting point of about 140° F. This composition should be applied to the fabric at a temperature of about 225° F., to 95 insure that it will thoroughly penetrate all the pores and interstices of the fabric and completely impregnate and saturate it. The fabric so treated is illustrated by the reference character B in the drawing. To one 100 side of this fabric is applied a layer or ply of material, indicated in the drawing by the character A, which is impervious to and unacted upon by "gas drip" or organic solvents. For this material may be employed 105

110

any one of the following which are mentioned as examples: A parchment or parchmentized fabric such as parchmentized paper or vegetable tissue obtained by treating 5 paper, vegetable fiber or the like with sulfuric acid or other parchmentizing substances; or, the ply A may consist of a colloidal cellulosic layer, film or sheet, such for instance as viscose; or the ply A may consist 10 of a chromatized gelatinous layer such as chromatized glue or similar gelatinous substances which upon an exposure to light becomes insoluble and impervious to organic solvents including "gas drip"; the gelatinous substance may also be tannated, that is, 15 treated with tannic acid instead of chromatized. I have found a parchmentized tissue or sheet such as parchmentized paper employed for the layer A, to give good results; 20 but any of the other materials mentioned may be employed without departing from the invention.

The layer or ply A is united to the fabric B in any desired manner as by rolling the 25 two plies A and B together as the latter issues from the saturating tank by pressing the same between rollers, or the layer A may be spread upon the treated fabric B and rolled thereon when its nature is such as to 30 permit this mode of operation.

Fig. 3 in the drawing illustrates one of the simplest forms of the invention and shows a fabric made up of the layers B and A treated and united as above described and an exterior 35 layer C which is composed of a bituminous or asphaltic composition having a higher melting temperature than that used for layer B. The composition employed for the layer C should have a melting temperature of about 300° F., and may be applied at 40 a slightly higher temperature. For ordinary purposes the fabric according to my invention is of the structure shown in Fig. 4 in which the "drip" proof material or layer 45 A forms a middle ply or layer between two plies or layers B—B, of waterproof material, one on each side thereof, and an outer layer of the asphaltic composition C.

In order to give the material the property 50 of adhering to the surfaces when it is applied, one or both faces is provided with a coating of sand or fine gravel or broken stone, grit or the like which is partially embedded in the outer layer C leaving portions of the sand 55 particles protruding from the face of the layer. This mineral facing is illustrated by the reference character D. This mineral facing of sand or the like is preferably applied in a heated condition to the surface of the fabric 60 by sprinkling the same thereon and pressing the same therein. By providing the fabric with a facing of this character it may be readily made to adhere to any cement or concrete

surface. The fabric is applied to such surface when the latter is green or soft. It will 65 firmly adhere to a wet or "green" cement or concrete surface, the protruding portions of the sand or mineral particles being embedded in the soft cement or concrete, by pressing or rolling in contact therewith and when the 70 cement is set or hardened the adhesion between the fabric and the cement is perfect. The fabric may be applied to a hardened cement concrete or any other surface by applying a layer of Portland or hydraulic cement 75 to the surface and spreading the fabric thereon. The projecting portions of the mineral particles form a bonding surface for the fabric which unites with the cement wall or other surface to which it is applied. 80

The fabric may if desired be made after the manner illustrated in Fig. 2 in which are shown two plies or layers of a drip proof material A, one on each side of a water proof fabric B. It will be understood that as 85 many plies of drip proof material may be employed as is desired or necessary and the fabric may be built up of alternate layers of water proof fabric and "drip" proof materials. The outer facing of sand or the like may of course be omitted if desired.

What I claim is:—

1. A waterproofing material having in combination a fabric or ply impregnated with a waterproof bituminous composition and a 95 layer or ply of parchmentized cellulose.

2. A waterproofing material having in combination a fabric or ply impregnated with a waterproof bituminous composition, a 100 layer or ply of parchmentized cellulose and an outer coating of a pliable bituminous composition.

3. A waterproofing material having in combination a plurality of layers of fabric impregnated with a bituminous waterproof composition, an intermediate layer of parchmentized paper and an outer coating of bituminous waterproof composition. 105

4. A water proofing material having in combination a layer or ply of fabric impregnated with a bituminous waterproof composition, a layer or ply of parchmentized cellulose and an outer bonding surface formed of mineral particles protruding therefrom. 110

5. A waterproofing material having in combination a layer or ply of fabric impregnated with a bituminous waterproof composition, a layer or ply of parchmentized paper, an outer coating of bituminous composition 115 and a bonding surface of mineral particles 120 partially embedded in said outer coating and protruding therefrom.

JOHN GLASSFORD.

Witnesses:

E. R. MINER,

HENRY C. WORKMAN.